

United States Patent [19]  
Herrnring

[11] 3,837,750  
[45] Sept. 24, 1974

[54] SOCKET STRUCTURE FOR THE BALL OF  
A BALL POINT PEN REFILL

849,432 8/1960 Great Britain ..... 401/216

[75] Inventor: Heinz Günther Herrnring,  
Alveslohe, Germany

Primary Examiner—Lawrence Charles  
Attorney, Agent, or Firm—Walter Becker

[73] Assignee: Montblanc-Simplo GmbH,  
Hamburg, Germany

[22] Filed: June 4, 1973

[57] ABSTRACT

[21] Appl. No.: 366,855

A socket structure for a ball point refill, which comprises a ball made of corundum and arranged inside an outer supporting shell provided in its interior with a compound bearing consisting of a backing shell having a hardness exceeding 800 kg/sq.mm Vickers and an inner lining facing the ball and having a hardness of less than 200 kg/sq.mm Vickers.

[56] References Cited

FOREIGN PATENTS OR APPLICATIONS

1,108,400 8/1955 France ..... 401/216

4 Claims, 1 Drawing Figure



PATENTED SEP 24 1974

3,837,750



## SOCKET STRUCTURE FOR THE BALL OF A BALL POINT PEN REFILL

The invention relates to a socket for the ball of a ball point pen refill comprising a multi-layer bearing socket having an outer supporting shell consisting of a high strength material having a high yield point in conjunction with an inner electrolytically or chemically deposited bearing liner consisting of chromium, nickel or an alloy containing one of these metals and having a hardness exceeding 600 kg/sq.mm Vickers.

Sockets of this kind have in the past given a satisfactory account of themselves. However, in the meantime metal compositions have become known which permit the quality and wearing properties of the writing points of ball point pen refills to be even further improved.

It is therefore the object of the present invention to provide a writing point for a ball point pen refill which excels by its quality as a writing point and by its long useful life.

According to the invention this is achieved by providing a ball made of corundum contained in a compound bearing inside an external supporting shell, said compound bearing comprising a backing shell exceeding 800 kg/sq.mm Vickers in hardness, whereas an inner lining facing the ball is softer than 200 kg/sq.mm Vickers.

In a preferred embodiment of the invention the external supporting shell which exceeds the ball in size is provided with an electro-deposited nickel-tin layer which serves as a backing shell upon which a soft layer of silver is deposited to provide the inner lining.

The combination of the proposed ball with a compound bearing firstly ensures excellent dimensional stability throughout the life of the point of the refill. On the other hand, the soft inner lining gives a soft writing touch.

Other details and features of the invention will become apparent from the following specification in connection with the accompanying Drawing illustrating a longitudinal section through the point according to the invention of a ball point pen refill.

The socket for the ball 1 of a ball point pen refill comprises substantially an outer supporting shell 2, a backing bearing shell 3 and an inner lining shell 4. The material used for the inner shell 4 should have a hardness of less than 200 kg/sq mm Vickers, preferably between 80 and 120 kg/sq mm Vickers. The outer supporting shell 2 may be made of a substance selected from the group consisting of chromium, nickel, and an alloy containing at least one of the metals chromium and nickel and having a hardness in excess of 600 kg/sq mm Vickers. Such alloys may e.g., be:

- a. A chromium-iron alloy having from 10 to 20 percent by weight of iron and the remainder chromium.
- b. A chromium-tungsten alloy having from 30 to 40 percent by weight of tungsten and the remainder chromium.
- c. A nickel-chromium alloy having from 0.1-5 percent by weight of chromium and the remainder nickel.
- d. A tin-nickel alloy having from 10 to 70 percent by weight of tin and the remainder nickel.
- e. A nickel-aluminum oxide alloy having from 0.1-10 percent by volume of  $\text{Al}_2\text{O}_3$  and the remainder nickel.

f. A nickel silicon carbide alloy having from 1-50 percent by volume of silicon carbide and the remainder nickel.

It is, of course, to be understood that the above alloys may have minor negligible impurities.

The backing bearing shell 3 is applied to the supporting shell 2, a material being used for shell 3 which has a hardness in excess of 600 kg/sq. mm Vickers, when a single phase smooth hard layer is involved. When a multi-phase layer is involved, the hardest phase has a hardness in excess of 1,000 kg/sq. mm Vickers. To this end, a nickel-tin layer is electro-deposited onto the interior of the supporting shell 2. A large number of blanks for the points of ball point pen refills are thus treated in this way simultaneously. They are inserted from below into the upper part of a holder. The individual holes in the upper part for the reception of the points are fitted with sealing rings. This upper part contains a heating chamber through which all the inserted points pass. The heating chamber is connected by two pipes to a heat source. Principally this will be a source of hot steam.

A bottom part which contains a hole for the reception of each point is now attached to the upper part. Each hole is open at its bottom end which has a reduced diameter. This end may also be a convergent cone. Seals between the points on the one hand and the upper and lower parts on the other hand ensure that the assembly formed by the upper and lower parts can be immersed in a bath without causing the exteriors of the points to be wetted.

For performing the electro-deposition the assembly is suspended in a bath and vertically oscillated, preferably in the axial direction of the points. A bearing shell 3 will thus be deposited inside the outer supporting shell.

In order even further to improve the properties of the socket in the ball point pen refill the invention further proposes to deposit on the hard film of the backing shell 3 a further soft lining having a hardness of less than 200 kg/sq. mm. This softer layer consists of silver and improves the "running-in" properties besides lengthening the life of the bearing. For this purpose a silver layer is selected which is free from hardening additives, for instance free from antimony, and which is deposited from a silver bath containing cyanide potassium hydroxide. The same method may be employed as that above described for applying the backing shell 3.

The finished ball point, into which the ball 1 has been inserted can finally be subjected to a thermal treatment in vacuo or in a protective, i.e., inert atmosphere. This post thermal treatment consists in a heat treatment for an hour in a vacuum or in an inert atmosphere at a temperature of from 200° to 500° centigrades, preferably at a temperature of from 250°-300° centigrades. The thermal treatment improves the bond between the several layers by fusion. The properties of the bearing may thus be further improved. However, when the ball 1 is located by pinching the edges of the shells, allowance must be made for the contraction caused by the thermal treatment. The ball 1 must therefore be inserted prior to the heat treatment with a slightly greater clearance.

It is, of course, to be understood, that the present invention is, by no means, limited to the specific showing

in the drawing, but also comprises any modification within the scope of the appended claims.

What I claim is:

1. For use in connection with a ball point refill writing instrument, the combination of: a multi-layer bearing socket having an outer supporting shell comprising a substance selected from the group consisting of chromium, nickel, and an alloy containing at least one of the metals chromium and nickel and having a hardness exceeding 600 kg/sq.mm Vickers; a ball made of corundum and arranged inside said outer supporting shell; a compound bearing arranged on the inside of said outer supporting shell and comprising both a backing shell having a hardness exceeding 800 kg/sq.mm Vickers; and also an inner lining adjacent to and directly facing said ball and having a hardness of less than 200 kg/sq.mm Vickers.

2. A combination according to claim 1, in which the external supporting shell is of slightly greater dimensions than said ball and is provided with an electro-deposited nickel-tin layer forming said backing shell and with a soft silver film deposited on said backing shell and forming said inner bearing lining directly for

said ball.

3. A combination according to claim 1, in which said outer supporting shell consists of a heterogeneous aluminum multi-component bronze predominantly of copper.

4. In a method of treating a ball point refill having: a multi-layer bearing socket with an outer supporting shell comprising a substance selected from the group consisting of chromium, nickel and an alloy containing at least one of the metals, chromium and nickel, and having a hardness exceeding 600 kg/sq.mm Vickers, a ball made of corundum and arranged inside said outer supporting shell, and comprising a backing shell having a hardness exceeding 800 kg/sq.mm Vickers, and an inner lining in the form of a soft silver film adjacent to and facing said ball and having a hardness of less than 200 kg/sq.mm Vickers, which includes the step improvement of: subjecting said ball point refill to a heat treatment so as to create both a good bond between the several shells and an increase in the hardness of said supporting shell by diffusion, and also a reduction in the hardness of said silver film.

\* \* \* \* \*